

**1**

3,352,639

**PROCESS FOR THE OXIDATION OF  $TiCl_4$   
TO PRODUCE  $TiO_2$** 

John Peter Wikswo, Ridge Drive, Va., assignor to American Cyanamid Company, Stamford, Conn., a corporation of Maine  
No Drawing. Filed Feb. 17, 1965, Ser. No. 433,491  
10 Claims. (Cl. 23—202)

**ABSTRACT OF THE DISCLOSURE**

The present invention relates to an improved method of preparing  $TiO_2$  by the reaction of titanium tetrachloride and relatively pure carbon monoxide with oxygen in the presence of a small amount of hydrogen sulfide. This invention is based upon the discovery that hydrogen sulfide in relatively small amounts, not only exerts a catalytic effect upon the reaction, but also produces an additional beneficial effect beyond that produced by water alone and that it does this without the undesirable hydrolysis of the feed materials occurring when water alone is used.

This invention relates to an improved method of burning  $TiCl_4$  to produce  $TiO_2$  pigment.

In the manufacture of  $TiO_2$  pigment by the combustion of  $TiCl_4$ , it is known that a small amount of water will serve to nucleate the formation of  $TiO_2$  pigment particles. As to such systems, it was found by previous workers that at least .05% by volume of water, based on the total combustion mixture, shall be used in order to obtain a beneficial nucleating effect. However, these findings have been discovered in connection with what is commonly referred to as a turbulent-type burner. Contrary to what might be expected, it was found that a beneficial effect could result from using water in amounts less than 0.05% in a combustion system involving a laminar flame burner of the type described in U.S. Patent No. 3,121,641. One significant difference between the two systems is that in the laminar flame burner, CO is one of the ingredients of the combustion feed mixture which serves to furnish additional heat to that generated by the combustion of  $TiCl_4$  to  $TiO_2$ . Further, in a laminar flame burner, the relatively smaller beneficial amounts of water, viz., from .005% to .06% by volume, based on the total feed mixture, appear to catalyze the combustion of CO to  $CO_2$  and the heat thus evolved appears to have a beneficial effect on pigment formation. From these considerations, it is apparent that the nature of the reactions occurring in a turbulent-type burner is different from that taking place in a laminar-flow burner.

In a laminar-flame burner, it is customary to use screens in the feed inlets to create a laminar-flow condition. The presence of water in the feed may tend to hydrolyze the  $TiCl_4$  to produce a hydrolytic product that may tend to deposit on the screens of the feed tubes. The deposition of the hydrolytic product tends to interfere with the flow of the feed material, thus leading towards an undesirable condition. To avoid this tendency, additional materials were examined from the standpoint of determining how the combustion reaction could be benefited without the possibility of depositing hydrolytic product in the feed inlet. Quite unexpectedly, we have discovered that hydrogen sulfide in relatively small amounts not only exerts a catalytic effect but also produces an additional beneficial effect on the combustion reaction beyond that produced by water only and that it does this without the undesirable hydrolysis of the feed materials occurring in the burner inlet. Also, quite surprisingly, it was found from a series of experiments which led to the present dis-

**2**

covery that propane and HCl gave no beneficial effect in the laminar flame system, which illustrates that the benefit resulting from the use of  $H_2S$  involves a phenomenon other than merely forming  $H_2O$  in situ during the combustion reaction.

Accordingly, an object of this invention is to provide an improved method for the production of  $TiO_2$  pigment.

Another object of this invention is to provide a method of producing pigmentary  $TiO_2$  of an exceptionally high tint tone and tinting strength.

Other objects and advantages of this invention will become apparent from the following description and explanation thereof.

By means of the present invention, the feed mixture of  $TiCl_4$ , oxygen, aluminum chloride,  $H_2S$  and CO is fed to a laminar-flow burner under conditions suitable for the production of pigmentary  $TiO_2$ .

The combustion reaction is conducted at a temperature of about 1400° to 1850° C., and more usually about 1450° to 1600° C. The amount of CO present in the feed mixture is measured as a volumetric ratio of CO to  $TiCl_4$ , and in general, this ratio is about 0.1 to 3.0:1, more usually about 0.3 to 1.0:1. The total feed mixture being fed to the combustion zone is determined as a volumetric space velocity, i.e., the cubic feet per minute of feed mixture, measured at 25° C. at 1 atmosphere of pressure, per square foot of flow area in the feed mixture inlets leading to the burning zone. Generally, the volumetric space velocity is about 15 to 45, and more usually about 20 to 40. The combustion reaction takes place satisfactorily under essentially atmospheric pressure, however, a higher or lower pressure may be employed. The oxygen-containing gas, measured as the excess over the stoichiometric amount needed to react with all the  $TiCl_4$  (and assuming that a stoichiometric amount of oxygen is present to act with all the CO), is about 5 to 120% excess, on a volumetric basis, and more usually about 40 to 80% on the same basis. Aluminum chloride may also be present in the feed mixture in an amount of about 1 to 5% by weight, more usually about 2 to 3% by weight, measured as  $Al_2O_3$  in the  $TiO_2$  finished product. The amount of  $H_2S$  present in the feed mixture may vary from about .002 to .06% by volume, based on the total feed, and more usually .01 to .04% by volume on the same basis. Water may also be present in the feed mixture in an amount ranging from about .005 to .06% by volume, based on the total feed mixture, and more usually to .02 to .04% by volume on the same basis. The conditions described above for the reaction involving production of pigmentary  $TiO_2$  may be varied outside the ranges specified above without departing from the spirit of the invention.

In a laminar-flame burner of the type described in U.S. Patent No. 3,121,641, the feed material is divided into two main streams which are introduced into the burning zone from diametrically opposed directions. The combustion flames resulting from the burning of each stream oppose each other to form two adjacent continuous flame fronts which contact each other without significant intermixing between the materials of the undivided flames. The introduction of the feed mixture into the combustion zone may be accomplished in a variety of ways, however, in a commercial operation, it is preferred that dampening screens be present in the feed tubes of the burner system. The dampening screens reduce any tendency towards flow turbulence which may tend to occur from the passage of the gas within the confined area of the feed conduits. The feed mixture may be preheated to a temperature of about 180° to 300° C., more usually about 200° to 250° C. The oxygen-containing gas which is used in the combustion reaction may be either pure oxygen, air or enriched air. For reasons of efficiency of operation it is preferred

that pure oxygen be used as the source of oxygen for the reaction.

We have also discovered that large excesses of oxygen have a beneficial effect on the quality of the pigmentary  $TiO_2$ . The greatest benefit is obtained when using from about 80-120% excess oxygen. The excess oxygen appears to behave as a promoter of the  $TiO_2$  product, and con-

5 ing brick, which replaced the cooling jacket shown in the patent. The experiments were made using the reaction conditions shown in Table I below, including a reaction pressure of essentially one atmosphere. The apparatus and method of operation described in the patent are hereby incorporated by reference and made a part of the present specification.

TABLE I

| Run No.                                         | 1     | 2     | 3      | 4     | 5     | 6      | 7      | 8     | 9     |
|-------------------------------------------------|-------|-------|--------|-------|-------|--------|--------|-------|-------|
| $TiCl_4$ , <sup>1</sup> lb. mol/hr.             | 3.2   | 3.2   | 3.2    | 3.2   | 3.2   | 3.2    | 3.2    | 3.2   | 3.2   |
| Oxygen, molar excess                            | 80    | 80    | 80     | 80    | 80    | 80     | 80     | 80    | 80    |
| $CO/TiCl_4$ , molar excess                      | .55   | .55   | .55    | .55   | .55   | .55    | .55    | .55   | .55   |
| Vol. space velocity                             | 31    | 31    | 31     | 31    | 31    | 31     | 31     | 31    | 31    |
| $H_2O$ , Vol. percent (total feed) <sup>2</sup> | 0     | 0     | 0      | 0     | 0     | .0185  | .0185  | .0063 | .0063 |
| $H_2S$ , Vol. percent (total feed)              | 0     | .0061 | .0122  | .0184 | .0243 | .0063  | 0      | 0     | .0061 |
| Combustion Temp., °C.                           | 1,505 | 1,505 | 1,505  | 1,505 | 1,505 | 1,505  | 1,505  | 1,505 | 1,505 |
| Pigment quality, Tint Tone                      | V Br  | Br 2  | Br 1.3 | Br 1  | Br .3 | Br 1.5 | Br 2.6 | Br 7  | Br 7  |
| Tinting Strength                                | 1,200 | 1,680 | 1,650  | 1,705 | 1,670 | 1,675  | 1,650  | 1,470 | 1,680 |
| Pigment quality (ground): <sup>3</sup>          |       |       |        |       |       |        |        |       |       |
| Tint Tone                                       | V Br  | Br 1  | Br 0.5 | B11   | B11   | B11    | Br 2.2 | Br 6  | B11.0 |
| Tinting Strength                                | 1,310 | 1,740 | 1,745  | 1,775 | 1,760 | 1,740  | 1,740  | 1,575 | 1,770 |

<sup>1</sup>  $TiCl_4$  contains 3 mol percent  $AlCl_3$ .

<sup>2</sup> Where zero is indicated the  $H_2O$  was not more than .0002% by volume.

<sup>3</sup> Milled for 8 minutes in a 2-wheel Chaser Mill with 100 pounds of force on each wheel.

sequently it is possible to reduce the amount of aluminum chloride and/or water for the reaction by the use of such large excesses of oxygen. Without being bound by any theory, it appears that the large excess of oxygen creates a beneficial mass-action effect which makes possible reducing the amount of  $H_2O$  and  $H_2S$  which may be needed to obtain beneficial effects.

The  $H_2S$  may be added by a variety of methods to the total feed mixture. It can be added directly to the  $CO$  stream, which is later combined with the other ingredients of the feed mixture. Alternatively, it may be added to the vaporous mixture of aluminum chloride and  $TiCl_4$ . Generally, however, the  $H_2S$  is added to the  $CO$  stream in an amount of about 200 to 4000 p.p.m., and more usually about 600 to 1800 p.p.m. In any case, the amount of  $H_2S$  in the  $CO$  stream will be sufficient to provide the desired final concentration of  $H_2S$  in the total feed material.

When water is added to the reaction, it may be injected directly into the feed mixture or along with any one or more of the ingredients thereof. In commercial practice it is preferred that the  $CO$  stream be humidified in order to have an intimate association of the two materials. This can be accomplished by drying a wet stream of  $CO$  to the desired water concentration, or in the case of dry  $CO$ , the water can be added by passing the  $CO$  through a water tower. By whatever method is employed, generally the water content of the  $CO$  stream may be from about 400 to 4000 p.p.m., and more usually about 1200 to 1800 p.p.m. In any case, the amount of water present in the  $CO$  stream will provide the desired final water concentration in the total feed stream.

Aluminum chloride may also be added to the feed mixture containing  $TiCl_4$ . The aluminum chloride promotes the formation of rutile pigmentary  $TiO_2$ , and therefore is desirable for commercial practice. The aluminum chloride is first combined with  $TiCl_4$ . This may be done by vaporizing a mixture or solution of aluminum chloride and  $TiCl_4$  by heating the same to a temperature of about 140° C. to 250° C., more usually about 175° to 200° C., at a pressure of about 1 to 120 p.s.i.g., more usually about 20 to 45 p.s.i.g. The vaporous mixture of  $TiCl_4$  and  $AlCl_3$  may be readily combined with the other ingredients of the total feed mixture, such as  $CO$  and  $H_2S$  prior to entering the burner.

To provide a better understanding of the present invention, experiments were made in a burner of the type described in U.S. Patent No. 3,121,641, except that the burner tubes employed in the experiments reported below were 15 inches in diameter and the feed gases were introduced into the burner tubes without the tangential swirl. The hood of the burner was aluminum lined with insulat-

25 5 What is claimed is:

1. A process for producing titanium dioxide which comprises reacting titanium tetrachloride with an oxygen containing gas in the presence of a gaseous mixture consisting essentially of carbon monoxide and hydrogen sulfide, the hydrogen sulfide being present in an amount of about .002 to .06% by volume of the total gas, the volumetric ratio of carbon monoxide to titanium tetrachloride being about 0.1 to 3.0:1, at a temperature of about 1400° C. to 1850° C., the oxygen being employed in a stoichiometric excess of about 5 to 120% by volume, and a volumetric space velocity of the total gas being about 15 to 45.
2. A process for producing titanium dioxide which comprises reacting titanium tetrachloride with oxygen in the presence of a gaseous mixture consisting essentially of carbon monoxide and hydrogen sulfide, the hydrogen sulfide being present in an amount of about .01 to .04% by volume of the total gas, the volumetric ratio of carbon monoxide to titanium tetrachloride being about .3 to 1.0:1, at a temperature of about 1450 to 1600° C., the oxygen being employed at a stoichiometric excess of 40 to 80% by volume, and a volumetric space velocity of the total gas being about 20 to 40.
3. The process of claim 1 being further characterized by the additional presence of water in an amount of about .005 to .06% by volume of the total gas.
4. The process of claim 2 being further characterized by the additional presence of water in an amount of about .01 to .04% by volume of the total gas.
5. The process of claim 1 wherein the oxygen containing gas is oxygen.
6. The process of claim 2 being further characterized by the additional presence of about 1 to 5% aluminum chloride measured as  $Al_2O_3$  in the final pigment.
7. In a process of producing titanium dioxide by reacting titanium tetrachloride with an oxygen containing gas by means of diametrically opposed reactant streams to form two parallel laminar flames, the improvement which comprises reacting said materials in the presence of a gaseous mixture consisting essentially of carbon monoxide and hydrogen sulfide, the hydrogen sulfide being present in an amount of about .002 to .06% by volume of the total gas, the volumetric ratio of carbon monoxide to titanium tetrachloride being about .01 to 3.0:1, at a temperature of about 1400° to 1850° C., the oxygen being employed in a stoichiometric excess of about 5 to 120% by volume and a volumetric space velocity of the total gas being about 15 to 45.
8. In a process of producing titanium dioxide by reacting titanium tetrachloride with oxygen by means of

diametrically opposed reactant streams to form two parallel laminar flames, the improvement which comprises reacting said materials in the presence of a gaseous mixture consisting essentially of carbon monoxide and a small amount of hydrogen sulfide, the hydrogen sulfide being present in an amount of about .01 to .04% by volume of the total gas, the volumetric ratio of carbon monoxide to titanium tetrachloride being about 0.3 to 1.0:1, at a temperature of about 1450 to 1600° C., the oxygen being employed in a stoichiometric excess of about 40 to 80% by volume, and a volumetric space velocity of the total gas being about 20 to 40.

9. The process of claim 8 being further characterized by the additional presence of about .01 to .04% by volume of water.

10. The process of claim 8 being further characterized by the additional presence of water in an amount of .01 to .04% by volume of the total gas and about 1 to 5%

by weight aluminum chloride measured as  $Al_2O_3$  in the finished pigment.

#### References Cited

#### UNITED STATES PATENTS

|           |         |                |       |        |
|-----------|---------|----------------|-------|--------|
| 911,494   | 2/1909  | Hall           | ----- | 23—3.1 |
| 1,678,630 | 7/1928  | Bahr           | ----- | 23—3.1 |
| 1,807,528 | 5/1931  | Hiatt          | ----- | 23—3.1 |
| 2,635,946 | 4/1953  | Weber et al.   | ----- | 23—202 |
| 2,689,781 | 9/1954  | Schaumann      | ----- | 23—202 |
| 2,823,982 | 2/1958  | Saladin et al. | ----- | 23—202 |
| 2,957,753 | 10/1960 | Nelson et al.  | ----- | 23—202 |
| 3,069,282 | 12/1962 | Allen          | ----- | 23—202 |
| 3,121,641 | 2/1964  | Wiksmo et al.  | ----- | 23—202 |
| 3,224,836 | 12/1965 | Allen et al.   | ----- | 23—202 |

OSCAR R. VERTIZ, *Primary Examiner.*

EDWARD STERN, *Assistant Examiner.*